# EUROPEAN PATENT SPECIFICATION

(11) **EP 0 025 115 B1**
(45) Date of publication and mention of the grant of the patent: **14.09.1983**
(21) Application number: 80104567.5
(22) Date of filing: 01.08.1980
(51) Int. Cl.: D06N 5/00, E04D 5/02, E04D 5/10

(54) **High-strength roofing products using novel glass fiber mats; multiply systems and glass fiber mats per se**
Dachbahnen mit hoher Reissfestigkeit unter Verwendung von neuen Glasfaservliesen; Mehrschichtprodukte und Glasfaservliese an sich
Matériaux de couverture à haute ténacité à base de nouveaux feutres en fibres de verre; produits à plusieurs couches et feutres en fibres de verre en soi

(30) Priority: 30.08.1979 US 70991; 26.09.1979 US 79192
(43) Date of publication of application: 18.03.1981
(73) Proprietor: GAF CORPORATION, New York New York 10020 (US)
(72) Inventor: Bondoc, Alfredo A., Middlesex New Jersey 08846 (US)
(74) Representative: Grünecker, Kinkeldey, Stockmair & Schwanhäusser Anwaltssozietät

## Description

This invention relates to high-strength roofing products using novel glass fiber mats, and more particularly, to ashalt shingles and built up roofing products having exceptional tensile strengths.

Thin sheets or mats of glass fibers are finding Increasing application in the building materials industry, as for example, as felts in roofing products. These glass fiber mats are replacing base sheets made traditionally of cellulosic and/or asbestos fibers. Glass fiber mats usually are made commercially by a wet-laid process, which is carried out on modified paper-making machine, as described, for example, in the book by 0. A. Battista, Synthetic Fibers in Papermaking (Wiley 1964: N. Y.) A number of U.S. patents also provides a rather complete description of the wet-laid process and glass mats produced thereby, including 2,477,555, 2,731,066, 2,906,660, 3,012,929, 3,021,255, 3,050,427, 3,103,461, 3,108,891, 3,228,825, 3,634,054, 3,749,638, 3,760,458, 3,766,003, 3,838,995, 3,853,683, 3,905,067, 4,052,257, 4,112,174,4,129,674 and 4,135,029.

Unfortunately, however, none of these prior art glass fiber mats possess In combination, the high percentage of uniformly enmeshed individual filament fibers, small diameter voids, and high tensile strength properties which are desirable in application in roofing products, such as built-up-rooflng membranes or ply sheets. FR-A-2 204 582 and US-A-4 112 174 disclose a uniform fibrous mat consisting of a 2- fiber component system. The known mats are composed of both individual monofilament glass fibers of given fiber length and, in addition, a plurality of glass fiber bundles of elongated dimension whose filaments are held together in said bundles by a water insoluble system. According to the state of the art, the . increased mat strength is achieved by the presence of these elongated bundles.

EP-A-0 002 002 and EP-A-0 006 963 disclose the formation of a uniform fibrous mat in a wet-laid process. In this known process the glass fiber mat is made from a dispersion of glass fibers in an aqueous dispersant medium which includes as dispersant components an amine oxide or guar gum only as a dispersant.

Accordingly, it is an object of the present invention to provide a novel glass fiber mat, a high strength roofing product using this novel glass fiber mat, and a built up roofing system comprising multiple plies of said novel glass fiber mat as membranes and adhesive asphaltic coatings between said membranes.

A specific object of this invention is to provide a high tensile strength built up roofing membrane and system which includes a novel glass fiber mat which has at least 70% by weight of the fibers therein in the form of uniformly enmeshed individual filament fibers.

Another object of the invention is to provide such roofing products in which less than 20% of the area of the mat are voids which extend through the thickness of the mat, the rest being fibrous material.

A further object of the invention is to provide roofing products including glass fiber mats wherein at least 8096, 30% and 10% of the voids have an equivalent diameter whose size is correspondingly less than 50 micrometers, 10 micrometers and 5 micrometers, respectively.

Still another object herein is to provide such roofing products including a novel glass fiber mat with fibers having a length of 6.3 mm to 76.2 mm and a diameter of 3 to 20 micrometers, the mat including 70% to 90% glass fibers and 10% to 30% binder to hold the fibers together, and wherein the mat has a thickness of 0.1 mm. to 3 mm. and a basis weight of 20 glm2 to 200 g/m2.

Yet another object herein is to provide roofing products having glass fiber mats whose structure exhibits excellent tensile strength in both the machine and cross machine directions.

Among the other objects of the invention is to provide such roofing products having glass fiber mat whose porosity is suitable for impregnation of asphalt roofing shingles and built up roofing membranes and systems.
Figure 1 is a photograph of the glass fiber mat used in the roofing products of the present invention.
Figure 2 illustrates a built up roofing membrane of the invention.
Figure 3 shows a typical 3-ply composite built up roofing system of the invention.

In accordance with the objects of the invention, there is provided herein a novel glass fiber mat comprising glass fibers, voids extending through the thickness of said mat and a binder to hold said fibers together, said fibers having a length of 6.3 to 76.2 mm and a diameter of 3-20 micrometers said mat having a thickness of 0.1 to 3.0 mm and a basis weight of 20-200 g/m², which is characterised in that at least 70% by weight of said fibers are substantially of the same length and uniformly enmeshed individual filament fibers; less than 20% of the area of said mat are voids which extend through the thickness of the mat the rest being fibers, and at least 80%, 30% and 10% of said voids have an equivalent diameter which is less than 50, 10 and 5 micrometers respectively, the mat being formed by the wet laid process using a dispersion of said fibers in an aqueous dispersant medium including as dispersant components a derivatized guar gum including substituent groups attached to the guar gum and an amine oxide surfactant having the formula wherein R" R₂ and R₃ suitably are hydrocarbon groups containing 1-30 carbon atoms. There is further provided a high strength roofing product comprising this novel glass fiber mat and a bituminous material impregnated in said mat.

There is also provided a built up roofing system comprising multiple plies of said high strength built up roofing product and adhesive asphaltic coatings between said membranes. Referring now to the-drawings, Figure 1 shows a photograph of the glass mat used as a felt in the roofing products of the invention. The mat, generally referred to by reference numeral 10, includes a plurality of substantially uniformly enmeshed individual filament fibers 11 which comprise at least 70%, preferably 80% and optimally 90% or greater, by weight of the fibrous component of the mat. Less than 20% of the area of the mat are voids 12 which extend through the thickness of the mat, the rest being fibrous material. At least 80%, 30% and 10% of the voids have an equivalent diameter whose size is correspondingly less than 50 micrometers, 10 micrometers and 5 micrometers respectively.

The fibers suitably have a length of 6.3 mm to 76.2 mm and a diameter of 3 to 20 micrometers. The mat has a thickness of 0.1 to 3 mm., preferably 0.3 to 2 mm. and a basis weight, including a binder material to hold the fibers together, of 20 to 200 g./m². The fibrous material usually comprises 70% to 90% by weight of the mat, and the binder 10% to 30%. Any suitable binder substance may be used, which is usually a resinous material.

The following description of the formation of the roofing products of the invention, and of the glass mat used therein, will be made by reference to the wet-laid process, although, it will be understood that changes and modifications in the process conditions may be made within the skill of the art.

Accordingly, the wet-laid process of forming the mat comprises first forming an aqueous suspension or dispersion of a plurality of chopped bundles of glass fibers, each of which contains from 20 to 300 fibers per bundle, by intense agitation of the bundles in a dispersant medium in a mixing tank. The process is intended to filamentize or separate the fibers in the bundle within the aqueous dispersant medium. The dispersant composition then is fed through a moving screen on which the filaments enmesh themselves while water is being removed.

The dispersant medium includes a derivatized guar gum (hereinafter defined) in combination with a second dispersant component, suitably such as a tertiary amine oxide (also defined later). The glass fiber dispersion is made by first thoroughly mixing the derivatized guar gum in tap water to form a viscous mixture. Then the tertiary amine oxide constituent is added with stirring, and the chopped bundles of glass fibers are admixed to form the desired fiber dispersion composition.

After preparation of the stock glass fiber dispersion composition in this manner, the dispersion is pumped to a head box of a mat-forming machine where the desired glass mat is formed as a wet mat on the belt of the machine. A suitable binder then is applied to the formed mat, which is then dried, set and/or cured.

The derivatized guar gum component of the dispersion composition includes substituent groups attached to guar gum itself. Derivatized guars suitable for use herein are identified as such in the commercial products which are available from Stein, Hall and Co., Inc. Typical derivatized guars include Jaguar CMHP, which is a carboxymethylhydroxypropylated guar gum; C-13, which is a quaternary ammonium guar gum; and Jaguar HP-11, which is hydroxypropylated guar gum.

The amine oxide surfactant component of the dispersion composition is a tertiary amine oxide having the formula: where Rⱼ, R₂ and R₃ suitably are hydrocarbon groups containing between 1-30 carbon atoms. The hydrocarbon groups can be aliphatic or aromatic, and, if aliphatic, can be linear, branched or cyclic, and can be the same or different in each radical. The aliphatic hydrocarbon radical also can contain ethylenic unsaturation. Preferably, aliphatic groups are selected from among alkyl groups, such as lower alkyl or hydroxyalkyl groups having from 1-4 carbon atoms, and other substituted alkyl groups thereof, or long chain alkyl groups, having from 12-30 carbon atoms, such as stearyl, laurel, oleyl, tridecyl, tetradecyl, hexadecyl, dodecyl, octadecyl, nonadecyl, or substituted groups thereof, derived from natural or synthetic sources. The sum of the Rⱼ, R₂ and R₃ groups is 14-40 carbon atoms, and, most preferably, 18-24 carbon atoms.

Typical commercial amine oxides prepared for use herein include Aromox DMHT, which is dimethyl hydrogenated tallow amine oxide; Aromox DM16, which is dimethylhexadecyl- amine oxide; Aromox T/12, which is bis(2-hydroxyethyl) tallow amine oxide, available from Armak Co.; and Ammonyx SO, which is dimethylstearylamine oxide, available from Onyx Chemical Co.

A particularly useful amine oxide is Aromox DMHT, which has the formula: where R_{HT} is R_{T} hydrogenated to saturation, and R_{T} Is 3% tetradecyl, 27% hexadecyl, 16% octadecyl, 48% octadecenyl and 6% octa- decadienyl.

In order to further define a preferred mode of priming the mat of the invention the suitable, preferred and best mode parameters of such a process are given below in Table II. The following definitions apply to this data:
"Dispersion consistency" is the percent by weight of the glass fibers in the stock aqueous dispersion medium. "Formation consistency" is defined as the consistency of the fibers at the head box of the mat-forming machine, which may be the same or lower consistency than the dispersion consistency. The dispersion composition may be diluted with water before entering the head box; this "diluted formation consistency" is given in Table I. the "amine oxide concentration" is given in ppm of this component. The "derivatized guar gum concentration" is indicated as percent by weight of the composition.

Commercial glass fibers which form dispersions in the composition of the mat employed in the invention may be used herein, including, for example, glass fiber types E or C. Such fibers may be sized or unsized, and usable as dry or wet chopped form.

The glass mats produced in the process are uniform mats which have high tensile and tear strengths. For increased tensile strengths, generally, fibers of relatively lower diameters are used, while higher tear strengths are enhanced by using longer length and smaller diameter fibers.

The examples which follow will illustrate the invention, but are not to be considered as being limiting of the principles of practice thereof.

Most preferably, the basis weight of the finished mat (with binder) for built up roofing products should be at least 49 g/sq.m. and, optimally, 98 to 148 g/sq.m.

Suitably, these mats have a tensile strength in the machine direction (MD) of at least 300 N/50 mm. width, and in the cross-machine direction (CMD) of at least 100 N/50 mm. width, at a basis weight of 98 g/sq.m. Preferably, it has tensile strength values of 500 to 700 MD and 150 to 250 CMD. Optimally, the mats have a tensile strength of 800 MD and 300 CMD. Mats of isotropic tensile strength, wherein MD=CMD, may be used herein, and these mats exhibit tensile strengths of at least 100, preferably 300, and optimally, 500 N/50 mm. width.

These glass mats are used as felts in the manufacture of improved roofing products, in this invention, including roofing shingles, built up roofing membranes, and multi-ply systems, which are characterized by very high tensile and tear strengths.

The roofing products of the present invention may be made by conventional techniques. For example, a built up roofing membrane may be manufactured by coating the glass mat with hot bituminous material, which, optionally, may be admixed with a fine mineral filler, such as talc, mica or sand, thereby to impregnate the mat with the bituminous (asphaltic) material. Thereafter the membrane is cooled and wound into rolls.

For the manufacture of a roofing shingle product, generally the bituminous material is coated on both sides of the glass mat, and a layer of the material remains on the surfaces of the mat. Finally, roofing granules are applied to the bituminous material and adhered to the surfaces.

Referring now to Figure 2, there is shown the built up roofing membrane of the invention, referred to as 20. The membrane includes the glass mat 10 as a felt material which is impregnated with bituminous material 13.

Figure 3 shows a typical built up roofing system of the invention. The embodiment illustrated is a 3-ply system, generally indicated by reference numeral 30. The system is secured to a roof deck 14 covered by appropriate insulation 15 (optional), by means of a bituminous adhesive coating 16 or mechanical fasteners. The successive membranes are adhered to each other with bituminous coatings 16. The top membrane is also covered with a bituminous coating layer 17 which may include therein aggregate surfacing material 18. The top membrane, optionally, may be covered with suitable surface coatings, such as fibered aluminum roof coatings, cold applied solvent cutback, asphalt mastic and/or roofing granules.

### Example 1

### Preparation of glass mat

The mat-forming machine was a 0.5 m inclined wire Hydroformer which was adjusted to a processing condition to give a preferred fiber orientation in the machine direction (MD) over the cross machine direction (CMD). The dispersion composition consisted of Aromox DMHT, 20 ppm, CMHP, 0.2%, E-type glass fibers, 25 mm length, 16 micrometers diameter, sized, and wet chopped. The dispersion consistency was 0.5% the diluted formation consistency was lowered to 0.03 after dilution with additional dispersion composition removed during mat formation at the headbox.

The formed glass mat then is impregnated with ureaformaldehyde resin, and cured. The glass mat, with about 25% by weight binder had an excellent tensile strength, N/50 mm width, MD/CMD of 506/412, at a basis weight of 114 glm² and a thickness of 0.8 mm.

### Example 2

### Preparation of build up roofing membrane

The mat of Example 1 was impregnated with bituminous material having a softening point of about 104-110°C and a penetration test value (ASTM D5-65) at 25°C of about 16-18 millidecimeters. The impregnation was about 432%, based on the weight of the glass mat. The surfaces of the impregnated mat then were dusted with talc to prevent sticking upon rolling up the membrane. The tensile strengths MD/CMD, at 25°C., of the membrane were 686/525 N/50 mm. width, respectively. In use, this roofing membrane exhibits excellent high-strength and wear properties.

### Example 3

### Preparation of 3-ply built up roofing system

The membranes of Example 2 were unrolled and asphaltic adhesive material, (ASTM D312-71, Type III) was applied at a level usage of about 8.8 g/cm² between successive membrane layers. The tensile strength of this system was 56.3 kp/cm (CMD) at -18°C and 36 kp/cm (CMD) at +25°C.

## Claims

1. A glass fiber mat comprising glass fibers, voids extending through the thickness of said mat and a binder to hold said fibers together, said fibers having a length of 6.3 to 76.2 mm and a diameter of 3-20 micrometers said mat having a thickness of 0.1 to 3.0 mm and a basis weight of 20-200 g/m², characterised in that
a) at least 70% by weight of said fibers are substantially of the same length and uniformly enmeshed individual filament fibers,
b) less than 20% of the area of said mat are voids which extend through the thickness of the mat the rest being fibers, and
c) at least 80%, 30% and 10% of said voids have an equivalent diameter which is less than 50, 10 and 5 micrometers respectively,
the mat being formed by the wet laid process using a dispersion of said fibers in an aqueous dispersant medium including as dispersant components
A) a derivatized guar gum including substituent groups attached to the guar gum and
B) an amine oxide surfactant having the formula where Rⱼ, R₂ and R₃ suitably are hydrocarbon groups containing 1-30 carbon atoms.

2. A glass mat according to claim 1-wherein said individual filament fibres comprise at least 80% by weight of said fibers.

3. A glass mat according to claim 1 and/or 2 wherein said individual filament fibers comprise at least 90% by weight of said fibers.

4. A glass fiber mat according to any of claims 1-3 wherein the length of said fibers are 12.7 to 38.1 mm.

5. A glass fiber mat according to any of claims 1-4 wherein the diameter of said fibers are 8 to 19 micrometers.

6. A glass fiber mat according to any of claims 1-5 wherein said thickness of said mat is 0.3 to 2 mm.

7. A glass fiber mat according to any of claims 1-6 wherein said basis weight of said mat is 40 to 110 g/ₘ².

8. A glass fiber mat according to any of claims 1-7 wherein said fibers comprise 70% to 90% and said binder 10% to 40% by weight of said mat.

9. A glass fiber mat according to any of claims 1-8 wherein the tensile strength is at least 300/100 N/50 mm width MD/CMD, respectively, at a basis weight of 100 g/m^{2.}

10. A glass fiber mat according to any of claims 1-9 wherein at least 15% of said voids have an equivalent diameter which is less than 5 micrometers.

11. A glass fiber mat according to any of claims 1-10 having a fiber length of 25.4 mm, a fiber diameter of 16 micrometers, a mat thickness of 1 mm., a basis weight of 110 g/m², fiber and binder contents of about 80% and 20%, respectively, a tensile strength of 500/280 N/50 mm width MD/CMD, respectively, further characterised in that 85% by weight of said fibers are substantially uniformly enmeshed individual filament fibers, 18.4% by area of said mat are said voids, the rest being fibers, 82.9%, 37.0% and 17.9% of said voids having an equivalent diameter which is less than 50, 10 and 5 micrometers respectively.

12. A high-strength roofing product comprising:
(A) a glass fiber mat according to any of claims 1-11 and,
(B) a bituminous material impregnated in said mat.

13. A roofing product according to claim 12 wherein the diameter of said fibers is 12 to 19 micrometers.

14. A. roofing product according to claim 12 and/or 13 wherein said basis weight of said glass mat is 40 to 150 g/m².

15. A roofing product according to any of claims 12-14 wherein said fibers comprise 70% to 90% and said binder 10% to 30% by weight of said mat.

16. A roofing product according to any of claims 12-15 wherein the tensile strength of the glass mat is at least 300 and 100 N/50 mm width, MD and CMD, respectively.

17. A roofing product according to any of claims 12-16 wherein said product is a roofing shingle.

18. A roofing product according to any of claims 12-17 wherein said bituminous material also is present as a coating on both sides of said mat.

19. A roofing product according to any of claims 12-18 wherein in (A) said glass fibers have a fiber length of 25.4 mm, a fiber diameter of 16 micrometers, a glass mat thickness of 1 mm., a basis weight of 110 g/m², fiber and binder contents of 80% and 20% respectively, tensile strengths of 500 and 400 N/50 mm. width MD and CMD respectively, further characterised in that in a) 85% by weight of said fibers are substantially uniformly enmeshed individual filament fibers, in b) 18.4% by area of said mat are voids, the rest being fibers, in c) 82.9%, 37.0% and 17.9% of said voids having an equivalent diameter which is less than 50, 10 and 5 micrometers respectively.

20. A roofing product according to any of claims 12-19 in which said product is a membrane which is in rolled up form.

21. A built up roofing product according to claim 20 having a tensile strength of 500 to 700 MD and 150-to 250 CMD.

22. A product according to claim 20 wherein the tensile strength is 800 MD and 300 CMD.

23. A product according to claim 20 wherein the MD tensile strength is approximately equal to CMD tensile strength.

24. A product according to claim 20 wherein the tensile strength MD is at least 100, 300 or 500 N/50 mm.

25. A built up roofing system comprising:
a) multiple plies of said high-strength built up roofing product as defined in any of claims 12-24, and
b) adhesive asphaltic coatings between said membranes.

26. A system according to claim 25 having three plies of said roofing products.

27. A system according to claim 25 and/or 26 in which the bottom ply is secured to a roof deck with an additional adhesive asphaltic coating.

28. A system according to any of claims 25―27 in which said bottom ply is secured to a roof deck with a mechanical fastener.

29. A system according to any of claims 25-28 further characterised by including on said top ply an asphaltic top coating.

30. A system according to claim 29 in which said asphaltic top coating includes an aggregate surfacing material thereon.

31. A 3 ply roofing system according to any of claims 26―30 having a tensile strength CMD at -18°C of 56.3 kp/cm and 36 kp/cm CMD at +25°C, at a glass mat basis weight of 114 g/m2..

## Patentansprüche

1. Glasfasermatte, umfassend Glasfasern, sich über die Dicke der Matte erstreckende Poren und ein Bindemittel, um die Fasern zusammenzuhalten, wobei die Fasern eine Länge von 6,3 bis 76,2 mm und einen Durchmesser von 3 bis 20 Mikrometer besitzen und die Matte eine Dicke von 0,1 bis 3,0 mm und ein Grundgewicht von 20 bis 200 g/m² besitzt, dadurch gekennzeichnet, daß
a) mindestens 70 Gew.-% der Fasern einheitlich verstrickte, einzelne Filamentfasern von im wesentlichen gleicher Länge sind,
b) weniger als 20% der Mattenfläche Poren, die sich über die Dicke der Matte erstrecken, und der Rest Fasern sind,
c) mindestens 80, 30 bzw. 10% der Poren einen Äquivalenzdurchmesser von weniger als 50, 10 bzw. 5 Mikrometer besitzen,
wobei die Matte mittels dem Naßlegeverfahren (wet laid process) gebildet wird, unter Verwendung einer Dispersion der Fasern in einem wässrigen Dispersionsmittelmedium, umfassend als Dispersionsmittelkomponenten
A) einen derivatisierten Guargummi mit an den Guargummi gebundenen Substituentengruppen und
B) ein Aminoxid-Surfactans der Formel worin R₁, R₂ und R₃ geeigneterweise Kohlenwasserstoffgruppen mit 1-30 Kohlenstoffatomen darstellen.

2. Glasfasermatte nach Anspruch 1, dadurch gekennzeichnet, daß die einzelnen Filamentfasern mindestens 80 Gew.-% der Fasern ausmachen.

3. Glasfasermatte nach Anspruch 1 und/oder 2, dadurch gekennzeichnet, daß die einzelnen Filamentfasern mindestens 90 Gew.-% der Fasern ausmachen.

4. Glasfasermatte nach mindestens einem der Ansprüche 1 bis 3, dadurch gekennzeichnet, daß die Länge der Fasern 12,7 bis 38,1 mm beträgt.

5. Glasfasermatte nach mindestens einem der Ansprüche 1 bis 4, dadurch gekennzeichnet, daß der Durchmesser der Fasern 8 bis 19 Mikrometer beträgt.

6. Glasfasermatte nach mindestens einem der Ansprüche 1 bis 5, dadurch gekennzeichnet, daß die Dicke der Matte 0,3 bis 2 mm beträgt.

7. Glasfasermatte nach mindestens einem der Ansprüche 1 bis 6, dadurch gekennzeichnet, daß das Grundgewicht der Matte 40 bis 110 glm² beträgt.

8. Glasfasermatte nach mindestens einem der Ansprüche 1 bis 7, dadurch gekennzeichnet, daß die Fasern 70 bis 90 Gew.-% und das Bindemittel 10 bis 40 Gew.-% der Matte ausmachen.

9. Glasfasermatte nach mindestens einem der Ansprüche 1 bis 8, dadurch gekennzeichnet, daß die Zugfestigkeit mindestens 300 bzw. 100 N/50 mm Breite MD bzw. CMD bei einem Grundgewicht von 100 g/m² beträgt.

10. Glasfasermatte nach mindestens einem der Ansprüche 1 bis 9, dadurch gekennzeichnet, daß mindestens 15% der Poren einen Äquivalenzdurchmesser von weniger als 5 Mikrometer besitzen.

11. Glasfasermatte nach mindestens einem der Ansprüche 1 bis 10 mit einer Faserlänge von 25,4 mm, einem Faserdurchmesser von 16 Mikrometer, einer Mattendicke von 1 mm, einem Grundgewicht von 110 g/m², Faser- bzw. Bindemittelgehalten von etwa 80 bzw. 20%, einer Zugfestigkeit von 500 bzw. 280 N/50 mm Breite MD bzw. CMD, weiterhin dadurch gekennzeichnet, daß 85 Gew.-% der Fasern im wesentlichen einheitlich verstrickte, einzelne Filamentfasern sind, 18,4 Flächen-% der Matte aus den Poren und der Rest aus Fasern bestehen, 82,9, 37,0 bzw. 17,9% der Poren einen Äquivalenzdurchmesser von weniger als 50,10 bzw. 5 Mikrometer besitzen.

12. Hochfestes Bedachungsprodukt, umfassend:
A) eine Glasfasermatte nach mindestens einem der Ansprüche 1 bis 11 und
B) ein in die Matte einimprägniertes, bituminöses Material.

13. Bedachungsprodukt nach Anspruch 12, dadurch gekennzeichnet, daß der Durchmesser der Fasern 12 bis 19 Mikrometer beträgt.

14. Bedachungsprodukt nach Anspruch 12 und/oder 13, dadurch gekennzeichnet, daß das Grundgewicht der Glasmatte 40 bis 150 g/m² beträgt.

15. Bedachungsprodukt nach mindestens einem der Ansprüche 12 bis 14, dadurch gekennzeichnet, daß die Fasern 70 bis 90 Gew.-% und das Bindemittel 10 bis 30 Gew.-% der Matte ausmachen.

16. Bedachungsprodukt nach mindestens einem der Ansprüche 12 bis 15, dadurch gekennzeichnet, daß die Zugfestigkeit der Glasmatte mindestens 300 bzw. 100 N/50 mm Breite MD bzw. CMD beträgt.

17. Bedachungsprodukt nach mindestens einem der Ansprüche 12 bis 16, dadurch gekennzeichnet, daß das Produkt eine Dachschindel ist.

18. Bedachungsprodukt nach mindestens einem der Ansprüche 12 bis 17, dadurch gekennzeichnet, daß das bituminöse Material ebenso als Beschichtung auf beiden Seiten der Matte vorliegt.

19. Bedachungsprodukt nach mindestens einem der Ansprüche 12 bis 18, wobei.in (A) die Glasfasern eine Faserlänge von 25,4 mm, einen Faserdurchmesser von 16 Mikrometer, eine Glasmattendicke von 1 mm, ein Grundgewicht von 110 g/m², Faser- bzw. Bindemittelgehalte von 80 bzw. 20%, Zugfestigkeiten von 500 bzw. 400 N/50 mm Breite MD bzw. CMD aufweisen, weiterhin dadurch gekennzeichnet, daß in a) 85 Gew.-% der Fasern im wesentlichen einheitlich verstrickte, einzelnen Filamentfasern sind, in b) 18,4 Flächen% der Matte Poren und der Rest Fasern sind, und in c) 82,9, 37,0 bzw. 17,9% der Poren einen Äquivalenzdurchmesser von weniger als 50, 10 bzw. 5 Mikrometer aufweisen.

20. Bedachungsprodukt nach mindestens einem der Ansprüche 12 bis 19, dadurch gekennzeichnet, daß das Produkt eine Membran in aufgerollter Form ist.

21. Zusammengesetztes Bedachungsprodukt nach Anspruch 20 mit einer Zugfestigkeit von 500 bis 700 MD und 150 bis 250 CMD.

22. Produkt nach Anspruch 20, dadurch gekennzeichnet, daß die Zugfestigkeit 800 MD und 300 CMD beträgt.

23. Produkt nach Anspruch 20, dadurch gekennzeichnet, daß die MD-Zugfestigkeit ungefähr gleich der CMD-Zugfestigkeit ist.

24. Produkt nach Anspruch 20, dadurch gekennzeichnet, daß die Zugfestigkeit MD mindestens 100, 300 oder 500 N/50 mm beträgt.

25. Zusammengesetztes Bedachungssystem, umfassend:
a) mehrere Schichten des hochfesten, zusammengesetzten Bedachungsprodukts nach mindestens einem der Ansprüche 12 bis 24, und
b) haftende, asphaltische Beschichtungen zwischen den Membranen.

26. System nach Anspruch 25 mit drei Schichten des Bedachungsprodukts.

27. System nach Anspruch 25 und/oder 26, wobei die Unterschicht an einer Dachtragefläche mit einer zusätzlichen, haftenden, asphaltischen Beschichtung befestigt ist.

28. System nach mindestens einem der Ansprüche 25 bis 27, wobei die Unterschicht an eine Dachtragefläche mit einem mechanischen Befestigungsmittel befestigt ist.

29. System nach mindestens einem der Ansprüche 25 bis 28, dadurch gekennzeichnet, daß es weiterhin auf der Oberschicht eine asphaitische Deckbeschichtung umfaßt.

30. System nach Anspruch 29, wobei die asphaltische Deckbeschichtung ein gehäuftes Ober^{f}lächenbehandlungsmaterial (aggregate surfacing material) darauf umfaßt.

31. 3-Schichten-Bedachungssystem nach mindestens einem der Ansprüche 26 bis 30 mit einer Zugfestigkeit CMD bei -18°C von 56,3 kp/cm und 36 kp/cm CMD bei +25°C, bei einem Glasmattengrundgewicht von 114 g/m².

## Revendications

1. Natte de fibres de verre comprenant des fibres de verre, des vides s'étendant sur toute l'épaisseur de ladite natte et un liant maintenant les fibres assemblées, lesdites fibres ayant une longueur de 6,3 à 76,2 mm et un diamètre de 3 à 20 micromètres, la natte ayant une épaisseur de 0,1 à 3,0 mm et un poids par unité de surface de 20 à 200 g/m², caractérisé en ce que
a) au moins 70% en poids desdites fibres sont des fibres filamenteuses individuelles ayant sensiblement la même longueur et étant uniformément emmêlées,
b) moins de 20% de l'aire de ladite natte sont formés de vides qui s'étendent sur toute l'épaisseur de la natte, le reste étant formé de fibres, et
c) au moins 80%, 30% et 10% des vides ont un diamètre équivalent de moins de 50, 10 et 5 micromètres, respectivement, .
la natte étant formée par le procédé par voie humide en utilisant une dispersion desdites fibres dans un milieu dispersant aqueux comprenant comme composants dispersants
A) un dérivé de gomme guar portant des groupes substituants liés à la gomme guar et
B) un surfactant qui est un oxyde d'amine de formule: dans laquelle R,, R₂ et R₃ représentent avantageusement des groupes hydrocarbonés contenant 1 à 30 atomes de carbone.

2. Natte de verre suivant la revendication 1, dans laquelle lesdites fibres filamenteuses individuelles constituent au moins 80% en poids des fibres en question.

3. Natte de verre suivant la revendication 1 et/ou la revendication 2, dans laquelle les fibres filamenteuses individuelles constituent au moins 90% en poids des fibres en question.

4. Natte de fibres de verre suivant l'une quelconque des revendications 1-3, dans laquelle la longueur des fibres va de 12,7 à 38,1 mm.

5. Natte de fibres de verre suivant l'une quelconque des revendications 1 à 4, dans laquelle le diamètre desdites fibres est de 8 à 19 micromètres.

6. Natte de fibres de verre suivant l'une quelconque des revendications 1 à 5, dont l'épaisseur est de 0,3 à 2 mm.

7. Natte de fibres de verre suivant l'une quelconque des revendications 1 à 6, dont le poids surfacique est de 40 à 110 g/m².

8. Natte de fibres de verre suivant l'une quelconque des revendications 1-7, dans laquelle les fibres constituent 70 à 90% et le liant 10 à 40% en poids de la natte.

9. Natte de fibres de verre suivant l'une quelconque des revendications 1 à 8, dans laquelle la résistance à la traction est d'au moins 300/100 N/50 mm de largeur SM/STM, respectivement, pour un poids surfacique de 100 g/ₘ2.

10. Natte de fibres de verre suivant l'une quelconque des revendications 1 à 9, dans laquelle au moins 15% des vides ont un diamètre équivalent inférieur à 5 micromètres.

11. Natte de fibres de verre suivant l'une quelconque des revendications 1 à 10, ayant une longueur de fibres de 25,4 mm, un diamètre de fibres de 16 micromètres, une épaisseur de natte de 1 mm, un poids surfacique de 110 g/m², des teneurs en fibres et en liant d'environ 80% et 20%, respectivement, une résistance à la traction de 500/280 N/50 mm de largeur SM/STM, respectivement, caractérisée en outre en ce que 85% en poids desdites fibres consistent en fibres filamenteuses individuelles quasiuniformément emmêlées, 18,4% de la surface de ladite natte sont desvides, le reste étant composé de fibres, 82,9, 37,0 et 17,9% desdits vides ayant un diamètre équivalent qui est, respectivement, inférieur à 50, 10 et 5 micromètres.

12. Matériau de couverture de grande résistance mécanique, comprenant:
(A) une natte de fibres de verre suivant l'une quelconque des revendications 1-11 et
(B) une matière bitumineuse imprégnant la natte.

13. Matériau de couverture suivant la revendication 12, dans lequel le diamètre desdites fibres est de 12 à 19 micromètres.

14. Matériau de couverture suivant la revendication 12 et/ou la revendication 13, dans lequel le poids surfacique de la natte de verre est de 40 à 150 g/m².

15. Matériau de couverture suivant l'une quelconque des revendications 12 à 14, dans lequel les fibres constituent 70 à 90% et le liant 10 à 30% en poids de ladite natte.

16. Matériau de couverture suivant l'une quelconque des revendications 12 à 15, dans lequel la résistance à la traction de la natte de verre est d'au moins 300 et la largeur d'au moins 100 N/50 mm, SM et STM, respectivement.

17. Matériau de couverture suivant l'une quelconque des revendications 12 à 16, qui est un bardeau de toiture.

18. Matériau de couverture suivant l'une quelconque des revendications 12 à 17, dans lequel la matière bitumineuse est également présente comme revêtement sur les deux faces de la natte.

19. Matériau de couverture suivant l'une quelconque des revendications 12-18, dans lequel les fibres de verre dans (A) ont une longueur de fibres de 25,4 mm, un diamètre de fibres de 16 micromètres, avec une épaisseur de la natte de verre de 1 mm, un poids surfacique de 110 g/m², des teneurs en fibres et en liant de 80% et 20%, respectivement, des résistances à la traction de 500 et 400 N/50 mm de largeur, SM et STM, respectivement, caractérisé en outre par le fait que a) 85% en poids desdites fibres sont des fibres filamenteuses individuelles quasi uniformément emmêlées, dans b) 18,4% de l'aire de ladite natte sont formés de vides, le reste étant formé de fibres, dans c) 82,9%, 37,0% et 17,9% desdits vides ont un diamètre équivalent qui est inférieur à 50, 10 et 5 micromètres, respectivement.

20. Matériau de couverture suivant l'une quelconque des revendications 12 à 19, qui est une membrane sous la forme enroulée.

21. Matériau de couverture multicouche suivant la revendication 20, ayant une résistance à la traction de 500 à 700 SM et de 150 à 250 STM.

22. Matériau suivant la revendication 20, dans lequel la résistance à la traction est de 800 SM et de 300 STM.

23. Matériau suivant la revendication 20, dans lequel la résistance à la traction SM est à peu près égale à la résistance à la traction STM.

24. Matériau suivant la revendication 20, dans lequel la résistance à la traction SM est d'au moins 100, 300 ou 500 N/50 mm.

25. Système de couverture multicouche, comprenant:
a) des couches multiples dudit produit de couverture multicouche à haute résistance mécanique tel que défini dans l'une quelconque des revendications 12 à 24, et
b) des revêtements adhésifs bitumineux entre lesdites membranes.

26. Système suivant la revendication 25, comprenant trois couches desdits matériaux de couverture.

27. Système suivant la revendication 25 et/ou la revendication 26, dans lequel la couche inférieure est fixée à une dalle de toiture par un revêtement bitumineux adhésif additionnel.

28. Système suivant l'une quelconque des revendications 25-27, dans lequel la couche inférieure est fixée à une dalle de toiture à l'aide d'un élément mécanique de fixation.

29. Système suivant l'une quelconque des revendications 25-28, caractérisé en outre en ce qu'il comprend sur la couche supérieure une surcouche de revêtement bitumineux.

30. Système suivant la revendication 29, dans lequel la surcouche de revêtement bitumineux porte une matière de surface formée d'agrégats.

31. Système de couverture à trois couches suivant l'une quelconque des revendications 26-30, ayant une résistance à la traction STM à -18°C de 56,3 kp/cm et une résistance à la traction STM à +25°C de 36 kp/cm, pour un poids surfacique de la natte de verre de 114 g/m 2.
